

April 9, 1935.

I. J. NOVAK

1,997,308

FRICITION ELEMENT

Filed Feb. 15, 1932

Fig. 1.



Fig. 2.



Fig. 3.



Witness:

Stephen A. Pelosa

Inventor:  
Isador J. Novak.  
By Frank L. Belknap  
Attorney

## UNITED STATES PATENT OFFICE

1,997,308

## FRICTION ELEMENT

Izador J. Novak, Bridgeport, Conn., assignor to  
 Raybestos-Manhattan, Inc., Bridgeport, Conn.,  
 a corporation of New Jersey

Application February 15, 1932, Serial No. 593,023

3 Claims. (Cl. 188—251)

The present improvements relate more particularly to the production of brake linings of the hard formed segmental type wherein the binder comprises rubber or other suitable binder 5 in minor proportion to asbestos fibre.

It is well known in the art of making brake lining of the hard segmental type, wherein rubber or other suitable binder is used in minor proportion relative to the asbestos, to make up a 10 mixture of rubber, asbestos and solvent for the rubber, and to dry out the solvent and sheet the asbestos and rubber on a pair of horizontal rolls having even surface speed, one roll being heated and the other being cooled, whereby a sheet is 15 formed on the heated roll as the solvent dries out of the compound, and pressure is applied through the cold roll to densify the sheet. After the sheet is formed to the desired thickness, which, it may be added, is rarely above  $\frac{1}{8}$  of an inch, the rolls 20 are stopped, and the sheet is stripped from the hot roll.

Because of the fact that it is difficult to build up thicknesses substantially greater than  $\frac{1}{8}$  of an inch on rolls of this type, in making greater 25 thicknesses such as those used in brake lining, which range commonly between  $\frac{5}{8}$  and  $\frac{1}{4}$  of an inch, it has been necessary in the past to secure these thicknesses by laminating two or more sheets from the sheeting machine above described by means of rubber cement, or other cements. A type of segmental brake lining now 30 on the market comprises laminated sheet packing wherein sufficient sulphur is used with the rubber to produce hard rubber, and where the 35 laminated sheet packing is cut into strips of the desired developed length and width and is cured hard by heat while held to a curvature.

Another type comprises sheet packing wound 40 on a mandrel with fine brass wires and cementing material between the convolutions, the whole thereafter being cured hard while held under pressure. After cure, the segments are cut from the cylinder thus produced. It will be appreciated by those skilled in the art, that because of 45 the laminated structure necessarily inherent in brake linings made from these sheets, there is always the danger of delamination under the severe abuse encountered in use. Also, the cost of production necessarily includes the cost of 50 making sheet packing, which latter cost is high because of the fact that during one cycle, only a thin sheet may be produced. Furthermore, such rolls for making sheet packings are necessarily large in size, and must be held to accurate dimensions, which means high cost of installa-

tion and upkeep. Rolls 10 to 15 feet long and 3 to 5 feet in diameter are considered modern practice in producing sheet packing. Again, in order to make sheets of fair thicknesses on a sheet packing roll, that is, between  $\frac{1}{2}$  and  $\frac{1}{8}$  of an inch, a fairly long fibre asbestos is essential and such grades run from \$150.00 to \$300.00 per ton at the present time. By the method to be hereinafter described, short fibres ranging in cost from approximately \$30.00 to \$80.00 per ton are advantageously used, and long fibres are entirely unnecessary. Also, expensive sheet packing rolls are dispensed with entirely, and comparatively inexpensive equipment substituted. The development of the present invention contemplates the production of a single ply 10 unitary structure of unwoven asbestos with a binder comprising rubber or other suitable material whereby any desired thickness may be produced, and short fibre asbestos is used to advantage. Tapes made according to the present 15 invention are admirably suitable for the production of hard formed unwoven brake lining segments.

Among the advantages therefore, of the present 20 invention as compared with processes now in use for making this type of brake lining, is that the final product is a single ply unitary structure having no laminations or plies, which of course, eliminates danger of delamination. Another advantage is the speed of production due to the speed 25 with which an extruding machine can be operated as compared with present methods of manufacture. This, of course, is of importance from the standpoint of economy in labor cost per unit 30 manufactured, in addition to decreasing all of the costs entering into manufacturing. Another 35 incidental advantage resides in the use of an extruding machine costing comparatively little initially and to maintain and operate, as compared 40 with a set of sheeting rolls which have a high initial cost and expensive maintenance cost and which require skilled labor for operation. The use of an extruding machine also results in the advantage of not having an expensive machine 45 idle when it is necessary to shut down for any reason. This will be obvious from the fact that a battery of extruding machines can be purchased and operated for the relative cost of one set of sheeting rolls.

Another advantage is the flexibility of the asbestos fibre quality, there being a minimum fibre length as stated above which can be sheeted on sheet packing rolls, but there being no minimum 55 to the fibre length which can be extruded from

an extruding machine. In addition, the use of present process eliminates or substantially decreases the necessity for using rubber cement for plying, which is an expensive item in conventional processes of manufacture. Other objects and advantages will be apparent from the accompanying drawing and following detail description.

In the drawing, Fig. 1 is a top plan view of an extruded tape.

10 Fig. 2 is a sectional view taken on the line 2—2 of Fig. 1.

Fig. 3 is a sectional view taken on the line 3—3 of Fig. 1.

15 On one mode of carrying out this invention, compound of approximately the following composition is prepared by mixing in a Werner-Pfleiderer dough mixer:

|                               | Parts |
|-------------------------------|-------|
| Smoked sheet                  | 14.0  |
| 20 Litharge                   | 4.5   |
| Sulphur                       | 9.0   |
| Carbon black                  | 3.0   |
| Short asbestos fibre grade XX | 60.0  |
| Benzol                        | 126.0 |

25 It will be noted that I preferably use a low proportion of solvent for a reason which will be explained later. The above mixing necessarily further loosens up the asbestos fibres and distributes the fibres and other ingredients throughout the mass of the compound. The plastic mass resulting from the above mixing is fed into the hopper of a standard extruding or tubing machine such as is used in making rubber tubing, insulated wire, automobile treads, etc., which is provided with an orifice at the head so designed as to give the desired cross-section, preferably a tape 1 of about the width of the finished brake lining and a thickness of extruded tape which contains the necessary amount of solid material desired for the finished density. As the asbestos fibres obviously run in all directions throughout the mass of the material, when extruded, they run in all directions throughout the mass of the tape as shown best at 2 in Figs. 2 and 3. This is particularly advantageous because it makes a strong product, after the subsequent compression and hardening, i. e., stronger and less likely to separate into laminations than would be the case if the tape were built up in laminations or all the fibres ran parallel to the length of the tape. Also the sides of the die orifice smooth and surface trowel as it were, the surface of the tape resulting in a formation as shown best at 3 in Figs. 1 and 3. It will be seen that I am extruding a composition which

55 contains considerable solvent. On drying out this solvent, the residual solids are left in a porous but uniformly bound condition without breaks or laminations, and must later be compressed to allow for the pore space occupied by the solvent in designing the orifice of the tubing machine. With the above compound for a finished thickness of approximately .180", it is necessary to make a wet tape of approximately .343".

65 On leaving the head of the tubing machine, the extruded tape 1 may be taken up on a moving belt and carried through a heated drying chamber to remove the solvent, which, of course, may be recovered, if desired. At the end of the drying chamber, the partially or completely dried tape is fed into a takeup device which winds it into rolls of suitable diameter for easy handling. This step of winding the porous ribbon on a reel is of course, for convenience, and is not a necessary or essential step of the process.

If the drying is not complete at this point, the rolls should be placed in a drying oven and the stock dried until the solvent is completely removed. This, when a volatile solvent is used, is necessary to prevent blistering in later curing operation.

5 At this point, the product is a flexible spongy tape with the fibres in the interior running in all directions which must be further compressed to the required density for brake lining. This is 10 accomplished by passing the tape 1 through pressure rolls so gauged as to give the desired compression though of course, other means of compressing the tape may be employed. For instance, in the above stated example, it is approximately .343" thick and is compressed in these rolls to approximately .180", the density being approximately one oz. per cubic inch. Because of the nature of this composition, such compression takes place quite easily without substantial stretching or 20 distortion of the tape. Any such deformation strains in any direction are of course, resisted by the fibres which run in all directions.

15 After the tape 1 has been compressed to size, which may be as above described, or in a hydraulic press, it is cut into pieces of the desired developed length of the segment to be made. These pieces have now the exact width, length and thickness of the finished segment. They are now placed in curved forms of the desired 30 curvature and while so held, are subjected to heat sufficient to vulcanize the rubber or harden the other binder contained therein, which may be 275-325° F. more or less, for 1 to 4 hours, more or less, depending on the thickness of the finished 35 segment, the temperature and the types of binder and accelerator used.

25 In the above composition, the cure is approximately 3 hours at about 325° F. This may be materially shortened by the use of rapid rubber accelerators. The curing is accomplished ordinarily by placing the forms in heated ovens but it may also be advisable in some cases to conduct the cure in the ordinary type of heated mold under hydraulic pressure. The finished segment is now ready for application to brake shoes. It may or may not be machined on the surface, according to the accuracy desired. As a matter of fact, the above described process produces a 45 segment which is smooth and well within the 50 limits necessary for segmental brake linings of this type.

55 Because of the fact that it is a unitary mass of fibres, uniformly distributed throughout the mass and running in all directions therein, densely compacted and having no laminations, it gives very satisfactory results in service and shows no tendency to break down and disintegrate. Its tensile strength is of the order of 5000-6000 pounds per square inch and its hardness 21-25 60 Brinell, using a 500 kg. load on a 1 mm. ball. If the amount of solvent used is too great, two things will occur on attempting to extrude the composition: (1) The composition will not feed through the worm because of its slipperiness, and 65 (2) what material passes through the worm and through the head will show the effect of individual lumps of compound and there will be breaks and separated portions of extruded stock from which no satisfactory tape can be made. 70 In order to avoid this, it is necessary to limit the amount of solvent to such a quantity as will produce a solid extruded tape without breaks. It may also be desirable to introduce certain resinous materials such as oil-soluble phenol resin 75

which will increase the adhesion of the stock to the worm of the extruding machine. As an example of the latter, I have used the following composition with excellent results:

|                          | Parts |
|--------------------------|-------|
| Oil soluble phenol resin | 5     |
| Rubber                   | 10    |
| Litharge                 | 4.5   |
| Sulphur                  | 9     |
| 10 Carbon black          | 3     |
| XX asbestos fibre        | 60    |
| Benzol                   | 126   |

By the method above described, it will be noted that the production of the sheet material is entirely unnecessary in the process as is also lamination. The present process as carried out in the above described illustration, thus comprises essentially the formation of binder, asbestos, and solvent into tape having a desired cross-section, removal of the solvent, and the processing of the dried tape into condensed strips suitable for cure in forms to a required curvature. The economy of this method over the lamination of thin sheets prepared on costly machinery is obvious.

It may be found desirable to omit the last step in this process, that of curing in forms, and to substitute a partial cure to produce a flexible unwoven tape which may be marketed in rolls, as in the present flexible woven brake lining. This of course, would be included within the scope of the present invention.

It may also be advisable to introduce, either in conjunction with rubber or as binders in their own right, other materials such as phenol resins, stearin pitch, casein, cellulose-acetate, viscose, drying oils and the like. Any of these changes would of course, modify the handling of the extruded tape, but would not affect the intent of this invention, which is to provide an economical method of producing any desired thickness of asbestos, binder and solvent by extrusion through a predetermined orifice, where the nature of the compound is such that such extrusion could not take place except by the use of an extending solvent in considerable proportion. It is obvious to those skilled in the art that a mixture such as above designated without the use of a solvent would not be extruded because of the relatively small volume of rubber or other binder and asbestos, and because of the fact that asbestos, because of its fibrous nature, is very difficult to extrude without some means of extending it and preventing it from packing in the head of an extruding machine.

In the two illustrations given, I have cited the use of benzol as a solvent. It is to be understood

of course, that any other type of solvent suitable for the purpose may be employed. I do not wish to be limited to benzol. It is also to be understood that the relative proportions of constituents as well as the cited lengths, widths and thicknesses of the intermediate and final products set out in the specification are merely illustrative and may be varied widely within the scope of the invention. The subject matter of the present claims is also disclosed in a pending application by Abert and Whitelaw, No. 376-639, filed July 8, 1929, which has become Patent No. 1,932,919, assigned to the assignee of this application, Raybestos-Manhattan, Inc.

I have described in the above specification, the use of a standard tubing machine in which the force necessary for extrusion is developed by the action of a revolving worm on a plastic composition, but it is obvious that this force may also be developed in other mechanical devices, such as for example, a ram and cylinder, and it is to be understood that no limitation as to the type of extrusion apparatus is intended.

I claim as my invention:

1. A friction lining which will not de-laminate in use, which comprises a hard, dense body of fibrous asbestos and a hardened binder in the form of a continuous unlaminated strip of the cross section desired, the fibres on the surface exhibiting the greatest longitudinal positioning gradually becoming less marked as the fibres approach the center of the lining where the number of longitudinally placed fibres noticeably decreases relative to the surface.

2. A friction lining which will not de-laminate in use, which comprises a hard, dense body of fibrous asbestos and a vulcanized rubber in the form of a continuous unlaminated strip of the cross section desired, the fibres on the surface exhibiting the greatest longitudinal positioning gradually becoming less marked as the fibres approach the center of the lining where the number of longitudinally placed fibres noticeably decreases relative to the surface.

3. A friction material suitable for automobile brakes, clutches and the like, which comprises a hard, dense body of fibrous asbestos and a hardened binder in the form of a continuous strip of the cross-section desired, the fibres on the surface exhibiting the greatest longitudinal positioning gradually becoming less marked as the fibres approach the center of the lining where the number of longitudinally placed fibres noticeably decreases relative to the surface.

IZADOR J. NOVAK.